

# UNITED STATES PATENT OFFICE.

WALTER A. SCOTT, OF CHICAGO, ILLINOIS.

## CONCENTRATION PROCESS.

1,261,303.

Specification of Letters Patent.

Patented Apr. 2, 1918.

No Drawing.

Application filed August 27, 1917. Serial No. 188,810.

*To all whom it may concern:*

Be it known that I, WALTER A. SCOTT, a citizen of the United States, residing at Chicago, in the county of Cook and State 5 of Illinois, have invented certain new and useful Improvements in Concentration Processes, of which the following is a specification.

My invention is an improvement in the 10 flotation process of concentration wherein the metalliferous mineral is separated from the gangue by means of bubbles of air or other gas. As generally practised air is introduced into a freely flowing ore pulp 15 to which some so-called modifying agent such as an oil, either animal, vegetable or mineral, or some other substance such as coal or wood tar or derivatives thereof, or other substances either soluble or insoluble have 20 been added in suitable proportion. The air is generally introduced into the ore pulp either by mechanical agitation, which has the effect of beating the air into the pulp, or is introduced through the porous bottom 25 of the vessel in which the pulp is contained. Such processes are described in Patent No. 1,022,085 granted to J. M. Hyde April 2, 1912 and in Patent No. 1,201,934 granted to J. M. Callow October 17, 1916.

30 In practising the flotation process as above referred to it is necessary that the modifying agent be disseminated through the pulp and such dissemination has been accomplished by stirring or agitating the 35 pulp after the modifying agent is added.

I have discovered, however, that it is not necessary that the oil be mixed with the pulp but that the simple admixture of some vaporized oil with the air that is introduced 40 into the pulp effects the desired concentration. In using the term oil I include the various re-agents which have been used for the purpose of causing the gaseous bubbles to have a selective attraction for 45 the metalliferous mineral particles as distinguished from the particles of the gangue. I have now further discovered that it is not necessary to use any oils whatever in the process, that is, it is not necessary to 50 use any of the liquid substances heretofore employed in the flotation process, but that the concentration of the ore can be effected by the use of an admixture of air with a permanent gas. I use the term "permanent

gas" in the ordinarily accepted meaning of 55 a substance that remains gaseous under ordinary conditions as opposed to vapors which condense at ordinary temperatures. By ordinary temperatures I mean the ordinary temperatures of the atmosphere and of the 60 pulp which is subjected to the process. I have found that it is not necessary to conduct the process with gases that will condense under the conditions prevailing in the practice of the process, and that it is not 65 necessary to depend upon such a relation between the liquefying point of the gas and the temperature of the air or pulp as will cause the gas to assume a liquid form. On the contrary, permanent gases which persist 70 in the gaseous form at the prevailing temperature of the atmosphere and the pulp are effective in carrying out the flotation process.

For instance, a mixture of such a permanent gas with air when introduced into the ore pulp, either by the mechanical agitation method set forth in the Hyde patent above referred to, or when introduced into the pulp through a porous wall of the containing vessel, will effect concentration, causing 80 the metalliferous mineral particles to adhere to the bubbles and to be by them separated from the remainder of the pulp. For this purpose I prefer to utilize some hydrocarbon 85 gas, such as methane, or ordinary illuminating or fuel gas, but the choice of the particular gas to be used will, of course, depend upon the availability of different gases and their efficiency in connection with the particular ore to which the process is applied. 90

While the precise forces upon which the operation of my improved invention depends cannot be stated with absolute certainty, it appears most probable from such 95 investigations as have been made with the permanent gas which is mixed with the air, according to my invention, that the gas is adsorbed and forms a film at the interface between the gaseous contents of the bubble 100 and the surrounding pulp, such film having a higher degree of viscosity than the body of the pulp. Such adsorption of the permanent gas at the interface between the gaseous contents of the bubble and the water in the 105 pulp is not dependent upon condensation in the sense of liquefaction due to temperature, which fact in connection with the efficiency

of permanent gases leads strongly to the conclusion that the phenomenon depends upon adsorption. The viscous film thus formed at the interface likewise through the force of adsorption holds the metalliferous mineral particles as distinguished from the gangue particles, there being an attractive force due to adsorption between the viscous film and the metalliferous mineral particles, whereas no such force exists between the viscous film and the gangue particles. While this explanation is offered tentatively, it seems to afford the best theory now known and the one which best harmonizes with the facts.

The use of a permanent gas, as above described, is not dependent upon any particular method of carrying out the flotation process, but, on the contrary, is applicable for use in connection with any of the various modes in which flotation has heretofore been practised.

An example of the use of my improved process is the use of a mixture of acetylene and air used for the treatment of the zinc ore of the Butte & Superior Mining Company at Butte, Montana. In this operation a mixture of air and acetylene was supplied to the pulp through the porous bottom of the containing vessel with the result that the gaseous bubbles rising through the pulp effected concentration of the ore, the particles of zinc sulfid adhering to the bubbles and being by them carried to the surface in the form of a layer or column of bubbles which was overflowed from the vessel in the usual manner. By this means the ore was efficiently concentrated. The gas used, acetylene, is a permanent gas in the sense in which I herein use that term. The critical temperature of acetylene is about 37 degrees centigrade, the various authorities varying not over a fraction of a degree in their statements of this temperature. The critical pressure of acetylene is about 68 atmospheres, although the statements of this figure as given by different authorities vary to the extent of several atmospheres. The boiling point of acetylene at atmospheric pressure is in the neighborhood of -83 degrees centigrade, the authorities varying in the statement of this figure only to the extent of a fraction of a degree. It will be apparent, therefore, that under the conditions of temperature and pressure prevailing in ore concentration operations, acetylene is a permanent gas and is not subjected to conditions of temperature or pressure that would cause it to condense to liquid form. It is for this reason that I above referred to adsorption as the most probable explanation of the results obtained in practising my invention.

The selection of the particular permanent gas to be used in practising my invention

and the particular amount thereof to be used in admixture with air are, of course, dependent upon the nature of the ore pulp being treated. The proper regulation of these factors, that is, the most advantageous amount of the most efficient gas, or mixture of gases in admixture with air, can readily be determined by experimental operations upon any given ore, such experimental operations being necessary in the application of any process. My invention, therefore, includes the use of any one or more permanent gases in admixture with air and the adjustment of such mixture as to proportions of the different ingredients in such manner as to effect the best result in the separation of the metalliferous constituent of an ore, or of one or more metalliferous constituents of an ore from the other constituents. My invention further includes the use of permanent gases in connection with the several modes of procedure such as the introduction of gas by mechanical agitation and by introducing the gas through a porous medium into the pulp with resulting flotation of the metalliferous mineral, or without floating the metalliferous mineral, but merely transporting it by means of the bubbles to a segregated portion of the pulp where the bubbles are broken and their burden of metalliferous mineral permitted to settle. In the method last referred to the bubbles are broken as soon as they reach the surface either by means of pulsations of gas pressure above the surface of the pulp, by mechanical means, by a water spray or other convenient devices, and the bubbles upon being broken release the metalliferous mineral adhering to them, permitting it to settle. The operation is conducted in a vessel of such form that the bubbles in rising are deflected to a point outside of the main current of pulp flowing through the vessel whereby the mineral falling from the broken bubbles settles and is collected separately from the main stream of pulp flowing through the vessel.

Among the gases and gas mixtures which may be used are not only various gases which are chemical compounds, but also elementary gases and mixtures of the same.

While I have herein referred to admixtures of various permanent gases with air it will be obvious that the use of air is not indispensable inasmuch as other inert gases might be used in admixture with the permanent gases herein referred to, or such permanent gases or mixtures of them might be used under some conditions without any admixture of air, carbon dioxide or similar inert gas.

In the claims I use the expression "inert bubble-forming gas" to denote the gas, ordinarily air, whose principal function is that

of furnishing the larger part of the volume of the bubbles while being relatively inert in the matter of imparting to the bubbles the required degree of persistence and selective attraction for metalliferous mineral. Of course the word "inert" as used in the claims does not necessarily mean absolutely inert in the matter of the properties mentioned as under some conditions pure air bubbles may have some degree of selectivity and of course all bubbles have some degree of persistence. The "bubble-modifying gas" referred to in the claims is gas that in a practical and efficient degree imparts to the bubbles the necessary selectivity and persistence.

While my invention in its broad aspect is not restricted to any particular procedure for the introduction of the gaseous mixture into the pulp, or to any particular method of collecting the mineral that adheres to the bubbles, I have heretofore found it advantageous to introduce the gaseous mixture into the pulp through a porous medium thereby causing the building up of a column of bubbles and overflowing the upper part of the bubble column as in the process set forth in the Callow patent hereinbefore referred to.

30 What I claim is:

1. An ore concentration process comprising the operations of forming a mixture of an inert bubble-forming gas with a permanent bubble-modifying gas which when the mixture is introduced into a body of ore pulp causes the formation above the normal pulp level of a mass of bubbles to which certain of the mineral particles in the pulp adhere and others do not, introducing the mixture into an ore pulp, and separating the mineral adhering to the bubbles so formed from the remainder of the ore.

2. An ore concentration process comprising the operations of forming a mixture of an inert bubble-forming gas with a permanent bubble-modifying gas distilled from a non-gaseous substance which when the mixture is introduced into a body of ore pulp causes the formation above the normal pulp level of a mass of bubbles to which certain of the mineral particles in the pulp adhere and others do not, introducing the mixture into an ore pulp, and separating the mineral adhering to the bubbles so formed from the remainder of the ore.

3. An ore concentration process comprising the operations of forming a mixture of an inert bubble-forming gas with a permanent bubble-modifying gas distilled from an organic compound which when the mixture is introduced into a body of ore pulp causes the formation above the normal pulp level of a mass of bubbles to which certain of the mineral particles in the pulp adhere and others do not, introducing the mixture into

an ore pulp, and separating the mineral adhering to the bubbles so formed from the remainder of the ore.

4. An ore concentration process comprising the operations of forming a mixture of an inert bubble-forming gas with a permanent bubble-modifying gas which when the mixture is introduced into a body of ore pulp causes the formation above the normal pulp level of a mass of bubbles to which certain of the mineral particles in the pulp adhere and others do not, introducing the mixture into an ore pulp unmodified as to bubble forming tension, and separating the mineral adhering to the bubbles so formed from the remainder of the ore.

5. In a process of concentrating ores the operations of forming a mixture of an inert bubble-forming gas with a permanent bubble-modifying gas which when the mixture is introduced into an ore pulp causes the formation of a bubble column consisting of bubbles to which certain of the mineral particles in the pulp adhere and others do not, introducing said mixture into an ore pulp, causing the formation of a column of bubbles above the pulp, and separating the mineral adhering to the bubbles in the upper part of the bubble column from the remainder of the ore.

6. In a process of concentrating ores the operations of forming a mixture of an inert bubble-forming gas with a permanent bubble-modifying gas distilled from a non-gaseous substance which when the mixture is introduced into an ore pulp causes the formation of a bubble column consisting of bubbles to which certain of the mineral particles in the pulp adhere and others do not, introducing said mixture into an ore pulp, causing the formation of a column of bubbles above the pulp, and separating the mineral adhering to the bubbles in the upper part of the bubble column from the remainder of the ore.

7. In a process of concentrating ores the operations of forming a mixture of an inert bubble-forming gas with a permanent bubble-modifying gas distilled from an organic compound which when the mixture is introduced into an ore pulp causes the formation of a bubble column consisting of bubbles to which certain of the mineral particles in the pulp adhere and others do not, introducing said mixture into an ore pulp, causing the formation of a column of bubbles above the pulp, and separating the mineral adhering to the bubbles in the upper part of the bubble column from the remainder of the ore.

8. In a process of concentrating ores the operations of forming a mixture of an inert bubble-forming gas with a permanent bubble-modifying gas which when the mixture is introduced into an ore pulp causes the formation of a bubble column consisting of

- 4
- bubbles to which certain of the mineral particles in the pulp adhere and others do not, introducing said mixture into an ore pulp unmodified as to bubble forming tension, 5 causing the formation of a column of bubbles above the pulp, and separating the mineral adhering to the bubbles in the upper part of the bubble column from the remainder of the ore.
- 10 9. In a process of concentrating ores the operations of forming a mixture of an inert bubble-forming gas with a permanent bubble-modifying gas which when the mixture is introduced into an ore pulp causes the formation of a bubble column consisting of bubbles to which certain of the mineral particles in the pulp adhere and others do not, introducing said mixture through a porous medium into an ore pulp, causing the formation 15 of a column of bubbles above the pulp,
- 20

and separating the mineral adhering to the bubbles in the upper part of the bubble column from the remainder of the ore.

10. In a process of concentrating ore in the form of a pulp unmodified as to bubble-forming tension and contained in a vessel open to the atmosphere and having walls extending above the normal pulp level, the operations of introducing into said pulp through a porous medium a permanent gas 25 which when so introduced causes the formation of a bubble column consisting of bubbles to which certain of the mineral particles in the pulp adhere and others do not, and separating the mineral adhering to the bubbles 30 in the upper part of the bubble column from the remainder of the ore.

In testimony whereof, I have subscribed my name.

WALTER A. SCOTT.